

1

2,839,457

## ELECTROPLATING

Donald Gardner Foulke, Watchung, and Otto Kardos, Red Bank, N. J., assignors to Hanson-Van Winkle-Munning Company, a corporation of New Jersey

No Drawing. Application November 16, 1956  
Serial No. 622,530

5 Claims. (Cl. 204—49)

This invention relates to electroplating and, more particularly, to electrodepositing nickel from an aqueous acidic nickel plating bath. The invention is based on our discovery that aromatic N-oxide compounds, when incorporated in a nickel electroplating bath, particularly in conjunction with various sulfo-oxygen compounds, are capable of promoting the formation of excellent bright and ductile electrodeposits of nickel over a wide current density range.

The electrodeposition of nickel from a plating bath containing a sulfo-oxygen "carrier" brightener additive does not produce fully bright deposits. Moreover, such brightness as is produced using these agents is obtained over only a limited current density range. When, however, a small quantity of an aromatic N-oxide compound is incorporated in the plating bath together with a sulfo-oxygen compound, the brightening capacity of the bath is extended, and the electrodeposit is ductile and bright over a very wide current density range.

These aromatic N-oxide compounds possess, as their common structural feature, the presence of a highly polar nitrogen-oxygen bond, having the following structural formula:



Only relatively small quantities of the aromatic N-oxide compounds are required in the plating bath, especially when they are used in conjunction with a sulfo-oxygen "carrier" brightener, for we have found that the highly polar nitrogen-oxygen bond appears to exert a pronounced synergistic effect on the brightening capacity of the sulfo-oxygen compound. In general, concentrations of the aromatic N-oxide compounds as low as 0.01 gram per liter are effective. There appears to be no critical upper limit on the concentration of the N-oxide compound, but there is no advantage in using more than 1 gram per liter, and in most plating baths substantially full benefit of its presence is achieved with 0.5 gram per liter or less.

Any aromatic N-oxide compound which is capable of being dissolved by acid and does not undergo decomposition upon protonation may be selected for inclusion in the plating solution. We have obtained particularly satisfactory results by using a pyridine-N-oxide of the group consisting of pyridine-N-oxide, 2-picoline-N-oxide, 3-picoline-N-oxide, 4-picoline-N-oxide, 2,4-lutidine-N-oxide, 2,6-lutidine-N-oxide, 2,4,6-trimethylpyridine-N-oxide, 2-ethylpyridine-N-oxide, 3-ethylpyridine-N-oxide, and 4-ethylpyridine-N-oxide.

A preferred process according to this invention for producing bright nickel deposits comprises electrodepositing nickel from an aqueous acidic solution of at least one nickel salt, in which there is dissolved from about 0.02 to about 0.5 gram per liter of a pyridine-N-oxide compound having the formula



2

in which R<sub>1</sub>, R<sub>2</sub> and R<sub>3</sub> are substituents selected from the group consisting of hydrogen, methyl, ethyl and propyl radicals, and from about 1/4 to about 80 grams per liter of a water-soluble sulfo-oxygen compound of the group consisting of unsaturated aliphatic sulfonic acids, mono-nuclear and binuclear aromatic sulfonic acids, heterocyclic sulfonic acids, mononuclear aromatic sulfonic acids, the alkali metal, magnesium, ammonium, and nickel salts of said acids, and mononuclear aromatic sulfonamides and sulfonimides.

Preparation of the unsaturated N-oxide compounds may be accomplished by direct oxidation of the corresponding free base. The pyridine-N-oxide compounds generally are prepared by using a vigorous oxidizing reagent, such as ozone (O<sub>3</sub>), or the peroxy acids, such as peracetic acid, perbenzoic acid, and monoperphthalic acid. Examples of the pyridine-N-oxide compounds which may be used successfully in embodiments of this invention are listed in Table I. Although these unsaturated N-oxide compounds may be used in concentrations as high as 1 gram per liter, there is no particular advantage to be gained from the higher concentrations, and they are preferably used in the range of concentrations from about 0.2 to about 0.5 gram per liter.

TABLE I

Pyridine-N-oxide compounds



30  
35  
40  
45  
50  
55  
60  
65

| Compound                             | R <sub>1</sub>                | R <sub>2</sub>                | R <sub>3</sub>                | R <sub>4</sub>                | R <sub>5</sub>  |
|--------------------------------------|-------------------------------|-------------------------------|-------------------------------|-------------------------------|-----------------|
| Pyridine-N-oxide                     | H                             | H                             | H                             | H                             | H               |
| 2-Picoline-N-oxide                   | CH <sub>3</sub>               | H                             | H                             | H                             | H               |
| 3-Picoline-N-oxide                   | H                             | CH <sub>3</sub>               | H                             | H                             | H               |
| 4-Picoline-N-oxide                   | H                             | H                             | CH <sub>3</sub>               | H                             | H               |
| 2-Ethylpyridine-N-oxide              | C <sub>2</sub> H <sub>5</sub> | H                             | H                             | H                             | H               |
| 3-Ethylpyridine-N-oxide              | H                             | C <sub>2</sub> H <sub>5</sub> | H                             | H                             | H               |
| 4-Ethylpyridine-N-oxide              | H                             | H                             | C <sub>2</sub> H <sub>5</sub> | H                             | H               |
| 4-Isopropylpyridine-N-oxide          | H                             | H                             | C <sub>3</sub> H <sub>7</sub> | H                             | H               |
| 2,4-Lutidine-N-oxide                 | CH <sub>3</sub>               | H                             | CH <sub>3</sub>               | H                             | H               |
| 2,6-Lutidine-N-oxide                 | CH <sub>3</sub>               | H                             | H                             | H                             | OH <sub>3</sub> |
| 2-Methyl-5-ethylpyridine-N-oxide     | CH <sub>3</sub>               | H                             | H                             | C <sub>2</sub> H <sub>5</sub> | H               |
| 2-Methyl-4-isopropylpyridine-N-oxide | CH <sub>3</sub>               | H                             | C <sub>3</sub> H <sub>7</sub> | H                             | H               |
| 2-Methyl-4-ethylpyridine-N-oxide     | CH <sub>3</sub>               | H                             | C <sub>2</sub> H <sub>5</sub> | H                             | H               |
| 4-Methyl-3-ethylpyridine-N-oxide     | H                             | C <sub>2</sub> H <sub>5</sub> | CH <sub>3</sub>               | H                             | H               |
| 2,4,6-Trimethylpyridine-N-oxide      | CH <sub>3</sub>               | H                             | CH <sub>3</sub>               | H                             | CH <sub>3</sub> |
| 2-Ethyl-3,5-dimethylpyridine-N-oxide | C <sub>2</sub> H <sub>5</sub> | CH <sub>3</sub>               | H                             | CH <sub>3</sub>               | H               |

60  
65  
70

The compounds listed in Table II are examples of sulfo-oxygen compounds which, when used in the plating bath in combination with the unsaturated N-oxide compounds, extend the current density range over which the formation of ductile and bright nickel electrodeposits may be obtained. These sulfo-oxygen compounds may be used over a very wide range of concentrations (1/4 to 80 grams per liter) but preferably are used in an amount in the range from about 1 to about 20 grams per liter,



Excellent results were also obtained when the pyridine-N-oxides were used in a nickel sulfamate bath (Bath B) containing 15 grams per liter of sodium naphthalene-1,3,6-trisulfonate and 0.16 gram per liter of pyridine-N-oxide. The deposit formed from such bath in a Hull test cell was bright over a very wide current density range. Increasing the pyridine-N-oxide to 0.32 gram per liter did not substantially increase the brightness.

A nickel electrodeposit formed on the test panel from a nickel fluoborate bath (bath C) containing 15 grams per liter of sodium naphthalene-1,3,6-trisulfonate, but no pyridine-N-oxide compound, was hazy and only semi-bright. Upon the addition of 0.16 gram per liter of pyridine-N-oxide to this bath, the deposit was bright over the entire current density range. Similarly, bright deposits were obtained from fluoborate baths containing 15 grams per liter of sodium naphthalene-1,3,6-trisulfonate and from 0.16 to 0.26 gram per liter of 2,6-lutidine-N-oxide.

We claim:

1. The process for producing bright nickel deposits which comprises electrodepositing nickel from an aqueous acidic solution of at least one nickel salt in which there is dissolved from about 0.01 to about 1 gram per liter of an aromatic N-oxide compound possessing a polar nitrogen-oxygen bond having the structural formula



in which the nitrogen atom forms part of a heterocyclic ring, and from about  $\frac{1}{4}$  to about 80 grams per liter of a water-soluble sulfo-oxygen compound of the group consisting of unsaturated aliphatic sulfonic acids, mononuclear and binuclear aromatic sulfonic acids, heterocyclic sulfonic acids, mononuclear aromatic sulfonic acids, the alkali metal, magnesium, ammonium, and nickel salts of said acids, and mononuclear aromatic sulfonamides and sulfonimides.

2. The process for producing bright nickel deposits which comprises electrodepositing nickel from an aqueous acidic solution of at least one nickel salt in which there is dissolved from about 0.02 to about 0.5 gram per liter of a pyridine-N-oxide of the group consisting of pyridine-N-oxide, 2-picoline-N-oxide, 3-picoline-N-oxide, 4-picoline-N-oxide, 2,4-lutidine-N-oxide, 2,6-lutidine-N-oxide, 2,4,6-trimethylpyridine-N-oxide, 2-ethylpyridine-N-oxide, 3-ethylpyridine-N-oxide, and 4-ethylpyridine-N-oxide, and from about  $\frac{1}{4}$  to about 80 grams per liter of a water-soluble sulfo-oxygen compound of the group consisting of unsaturated aliphatic sulfonic acids, mononuclear and binuclear aromatic sulfonic acids, heterocyclic sulfonic acids, mononuclear aromatic sulfonic acids, the alkali-metal, magnesium, ammonium, and nickel salts of said acids, and mononuclear aromatic sulfonamides and sulfonimides.

3. The process for producing bright nickel deposits which comprises electrodepositing nickel from an aqueous acid solution of at least one nickel salt in which there is dissolved from about 0.01 to about 1 gram per liter of a pyridine-N-oxide having the formula



in which  $\text{R}_1$ ,  $\text{R}_2$  and  $\text{R}_3$  are substituents selected from the group consisting of hydrogen, methyl, ethyl, and propyl radicals, and from about  $\frac{1}{4}$  to about 80 grams per liter of a water-soluble sulfo-oxygen compound of the group consisting of unsaturated aliphatic sulfonic acids, mononuclear and binuclear aromatic sulfonic acids, heterocyclic sulfonic acids, mononuclear aromatic sulfonic acids, the alkali metal, magnesium, ammonium, and nickel salts of said acids, and mononuclear aromatic sulfonamides and sulfonimides.

4. An aqueous acidic nickel electroplating bath in which there is dissolved from about 0.02 to about 0.5 gram per liter of a pyridine-N-oxide having the formula



in which  $\text{R}_1$ ,  $\text{R}_2$  and  $\text{R}_3$  are substituents selected from the group consisting of hydrogen, methyl, ethyl, and propyl radicals, and from about  $\frac{1}{4}$  to about 80 grams per liter of a water-soluble sulfo-oxygen compound of the group consisting of unsaturated aliphatic sulfonic acids, mononuclear and binuclear aromatic sulfonic acids, heterocyclic sulfonic acids, mononuclear aromatic sulfonic acids, the alkali-metal, magnesium, ammonium, and nickel salts of said acids, and mononuclear aromatic sulfonamides and sulfonimides.

5. An aqueous acidic nickel electroplating bath in which there is dissolved from about 0.01 to about 1 gram per liter of a pyridine-N-oxide of the group consisting of pyridine-N-oxide, 2-picoline-N-oxide, 3-picoline-N-oxide, 4-picoline-N-oxide, 2,4-lutidine-N-oxide, 2,6-lutidine-N-oxide, 2,4,6-trimethylpyridine-N-oxide, 2-ethylpyridine-N-oxide, 3-ethylpyridine-N-oxide, and 4-ethylpyridine-N-oxide, and from about  $\frac{1}{4}$  to about 80 grams per liter of a water-soluble sulfo-oxygen compound of the group consisting of unsaturated aliphatic sulfonic acids, mononuclear and binuclear aromatic sulfonic acids, heterocyclic sulfonic acids, mononuclear aromatic sulfonic acids, the alkali-metal, magnesium, ammonium, and nickel salts of said acids, and mononuclear aromatic sulfonamides and sulfonimides.

#### References Cited in the file of this patent

#### UNITED STATES PATENTS

|    |           |        |               |
|----|-----------|--------|---------------|
| 50 | 2,644,788 | Shenk  | July 7, 1953  |
|    | 2,644,789 | Shenk  | July 7, 1953  |
|    | 2,647,866 | Brown  | Aug. 4, 1953  |
|    | 2,658,867 | Little | Nov. 10, 1953 |